

## UNITED STATES PATENT OFFICE.

JOE FRY, OF CANTON, MISSISSIPPI.

## LIQUID WAX FOR THREADS.

No Drawing.

Application filed January 27, 1925. Serial No. 5,144.

*To all whom it may concern:*

Be it known that I, JOE FRY, a citizen of the United States, and a resident of Canton, in the county of Madison and State of Mississippi, have invented certain new and useful Improvements in Liquid Wax for Threads, of which the following is a specification.

This invention relates to a wax particularly adapted for use in waxing threads and has for its object the provision of a fluid in which no ingredients are used which will soil fabrics or leather when secured together by threads treated with the liquid, but nevertheless will be effective for preserving and water-proofing the threads thereby preventing the usual breakage of the threads and a consequent separation of the sole and welt of a shoe.

20 A further object of the invention is the provision of a liquid wax for treating threads used in the manufacture of leather goods and for preserving the threads against ready breakage, the wax retaining its liquid state regardless of the temperature, and being of such consistency that the fibers of the thread will be thoroughly impregnated without leaving a surface coating which will mar the fabric when sewed.

25 This invention will be best understood from a consideration of the following detailed description; nevertheless it is to be understood that the invention is not confined to the disclosure, being susceptible of such changes and modifications which shall define no material departure from the salient features of the invention as expressed in the appended claim.

In carrying out my invention I have endeavored to produce a wax which will be free of rosin because the rosin tends to clog or corrode the various parts of the machine during the sewing operation, therefore the following ingredients and in the quantities

45 named are employed—

Parts.

|                                    |    |
|------------------------------------|----|
| Shoemaker's prepared machinery wax | 70 |
| Boiled linseed oil                 | 20 |
| 50 Banana oil                      | 5  |
| Oil of sassafras                   | 5  |

These ingredients are placed in a container and raised to the boiling point and maintained at such temperature until an intimate mixture is had and then the liquid is allowed to cool. It must be borne in mind that if the liquid thus produced is not of the proper density for certain purposes a greater quantity of shoemaker's wax may be added and the liquid boiled again. Where the density of the liquid is too great after cooling, boiled linseed oil may be added. The wax thus prepared will be maintained in a liquid state and used in the usual way with shoe machinery. Since the wax has been dissolved or thoroughly incorporated in the oils the wax will remain in solution and the product will present a liquid state.

55 The shoemaker's prepared machinery wax may be ordinarily described as being formed by melting together the best Swedish pitch and tallow in a vessel over a fire, the quantity of tallow being determined by experiment. The desired pitch is of a brown color when fractured.

60 The banana oil is introduced to prevent adhesion of the mixture to the machine. The oil of sassafras prevents any lumping of the wax, producing a smooth homogeneous mixture which thoroughly penetrates and saturates the thread, increasing flexibility and durability and prevents all staining and spotting of work so necessary where leather and fine fabrics are sewed together. This compound, as stated before, increases 65 the durability of the thread so that there is no ripping so long as there is any body to the leather at all.

70 What I claim is:

A liquid wax comprising the following: 75  
shoemaker's prepared machinery wax, 70 parts; boiled linseed oil, 20 parts; banana oil 5 parts and oil of sassafras 5 parts.

JOE FRY.